

Aug. 7, 1956

R. M. BAILLY ET AL

2,758,100

## DAIRY WAX COMPOSITION

Filed Jan. 2, 1952



1

2,758,100

## DAIRY WAX COMPOSITION

Randolph M. Bailly, Little Silver, and Harold F. Hitchcox, Cranford, N. J., assignors to Esso Research and Engineering Company, a corporation of Delaware

Application January 2, 1952, Serial No. 264,522

8 Claims. (Cl. 260—28.5)

This invention relates to a new and improved wax composition and more particularly relates to the use of such a composition in the coating of paperboard milk containers and the like. The invention is particularly concerned with the production of a high quality dairy wax composition produced by utilizing a relatively narrow cut paraffin wax fraction in conjunction with a relatively small amount of a material selected from the class consisting of microcrystalline waxes and polyethylene. The present application is a continuation-in-part of Serial No. 202,443, filed December 22, 1950, entitled "Improved Dairy Wax Composition," for Bailly et al., and now abandoned.

One of the objects of the invention is to coat or impregnate paperboard, particularly milk containers, with a wax composition having improved leakage resistance qualities in regard to the prevention of leakage through the cartons or liquid absorption into the cartons. Other objects of the invention will be set forth in the following description which illustrates preferred embodiments thereof, it being understood that the above statements of objects is made to explain the same without limiting it in any manner.

In the refining of hydrocarbon oils such as petroleum oils, it is known to segregate paraffin waxes from so-called paraffin distillates, waxy lubes and the like. The segregation of these waxes is secured by a number of processes. For example, it is known to chill the selected wax containing fraction in order to secure crystallization of the wax and to remove the wax crystals from the oil by filtering, centrifuging and the like. It is also known to use various dewaxing solvents such as liquid normally gaseous hydrocarbons, such as propane, as well as other solvents, such as methyl-ethyl ketone and the like. It is also known to utilize in dewaxing operations solvent mixtures wherein one solvent comprises a wax precipitating solvent while the other comprises a solvent having a high solubility for oil. A solvent mixture of this character, for example, comprises 60% by volume of toluene and 40% by volume of methyl-ethyl ketone. In utilizing a mixture of this character, it has been the practice to add the mixture in toto or incrementally to the waxy distillate as it is being chilled. In dewaxing operations, it is also known to use various filter aids and other agents in order to render the dewaxing and filtering operations more efficient.

The wax segregated from the hydrocarbon oil, usually termed "slack wax," contains from about 10% to 40% of

2

oil. The slack wax is refined usually by conventional sweating to produce "crude scale wax" in a manner to reduce the oil content to less than about 5% by weight. The slack wax may be distilled to obtain the desired boiling range wax prior to sweating, if desired. This "crude scale wax" generally has an oil content of about 2% to 3% by weight. In order to remove this oil from the scale wax to produce a refined wax having an oil content below about .5%, usually below about .3%, various procedures have been proposed and employed.

It is also known in the art to segregate microcrystalline waxes from residual oils. These microcrystalline waxes are of a relatively high melting point and of different crystalline structure. The microcrystalline or petrolatum waxes may be prepared from any of the paraffin or mixed base crude oils. The undistilled residue may be treated with sulfuric acid and neutralized to remove the tarry matter and unsaturated hydrocarbons. The undistilled residue also may be deasphalted. The treated stock, containing a fairly high percentage of wax, as evidenced by a very high pour point, may be dewaxed by blending with a dewaxing solvent, such as propane, methyl ethyl ketone-benzol, or petroleum naphtha and chilled, and filtered or centrifuged to separate the petrolatum wax from the oil solution.

This deoiling operation produces a wax containing some oil and solvent. The wax after removal of the solvent has a melting point of from about 140° to 180° F. The wax may be again put in solution with more solvent or naphtha and chilled and filtered or recentrifuged to further reduce the oil content. The wax which separates in either of these operations is referred to as crude petrolatum wax. The wax separated in the second deoiling process after stripping to remove solvent is fairly dry and of a low oil content. This wax should not be confused with petroleum jellies which contain large amounts of oil. The crude petrolatum wax may be again put into solution with naphtha and filtered through clay or an equivalent material in order to improve its color. The clay filtered solution is distilled to remove the naphtha, the residue being a refined petrolatum wax having a melting point within the range of about 140° to 180° F. The source of the crude oil and the oil content of the refined microcrystalline product will affect the melting point of the final wax product. The refined petrolatum wax, sometimes called amorphous wax, is of very small crystal structure.

The hereinbefore mentioned crude petrolatum wax may be fractionated into petrolatum waxes having melting points within the range of 140° F. to 180° F. Usually this separation is effected by fractional precipitation from ketone, propane or naphtha solutions. The terms "petrolatum waxes" or "microcrystalline waxes" are used in this application to cover the residual type petroleum waxes of very small crystalline structure, and having melting points above about 145° F. and oil contents in the range of about 1 to 10%.

In the paperboard carton art, moistureproofness and, where desired, liquidproofness have hitherto been attained through the use of paraffin wax. Paraffin, while inexpensive, has certain disadvantages. It is the general practice to apply the paraffin either to finished container blanks or to finished and erected containers, closed on one end,

Paraffin forms a relatively fragile coating subject to disruption when the paperboard is bent.

There has not hitherto been a satisfactory, cheap, coated paperboard for the manufacture of cartons or containers in which an interior coating provided the desired grease- and liquid-proofness, as hereinafter explained. The desirable qualities of such a product are these:

1. *Moisture- and liquidproofness.*—The coating should impart to the board a sufficiently high degree of resistance to penetration by (1) water vapor to prevent food products from drying out and becoming stale too rapidly and (2) liquids to insure satisfactory delivery to the consumer.

2. *Freedom from odor and toxicity.*—It is obvious that a coating for foodstuff containers should possess no odor nor any degree of toxicity.

3. *Airtightness.*—This quality is to be distinguished from resistance to moisture and liquids. The term "air-tightness" is used to mean the quality of blocking odors, whether the purpose be the protection of the contents of the container from contamination by foreign odors or the prevention of loss of aromatic values by the contents of the container.

4. *Low cost.*—Both the coating composition and its method of application should be such as to permit the lowest possible cost, since food products are distributed in large volume and are bulky in relation to dollar value. Hence, protection must be attained at the most economical level possible so as not to make it necessary to raise the selling price.

5. *Handleability.*—The coating imposed upon the paperboard should not be such as to interfere with the normal operations of producing cartons and containers. It must neither be so fragile as to be disrupted by normal handling operations, nor must it be tacky so as to make sheet separation difficult.

6. *Impact strength.*—Impact strength is a very important index to the suitability of waxes as coating materials. High impact strength, i. e., high resistance to deformation or cracking on impact, is related to the ability of the wax to withstand rough handling and chipping.

7. *Leakage resistance test.*—This test was developed to determine the ability of a wax to prevent leakage from paperboard milk cartons. It is based on a measurement of the percentage of leaking cartons which were subjected to a standardized impact by dropping on a bottom corner. A large sample size is chosen to increase the accuracy of the test by reducing the probable error resulting from a small percentage of non-standard quality cartons produced by the machine. This test is carried out as follows:

(a) 100 cartons which have been conditioned at least 24 hours at 73° F. and 50% relative humidity are coated and filled with 40° F. water on a standard milk carton machine in the normal manner.

(b) These cartons are stored 16 hours at 40° F.

(c) After storage, the cartons are individually dropped 5 inches on a standard corner. A device having a hinged lever arm and tripping mechanism is used to provide standard drops.

(d) Cartons that do not leak when dropped are stored for 24 hours at 40° F. and leakers noted. Any observed leakage is sufficient to call the carton a "leaker."

(e) The bottom gluing of all cartons are checked and any cartons with superior or inferior to "standard bottoms" are noted and their durability ratings discarded.

(f) The number of cartons that leak is expressed as a percentage of the group and reported as "per cent leakers."

8. *Storage tests.*—(a) *Absorption test at 73° F.*—Five empty, coated cartons are individually weighed-filled with a 1% solution of lactic acid, colored with methylene-blue, and stored at 73° F. for 72 hours. At the end of this period any leakers are noted and the "bulge" (average of

the widest portion of carton in both directions) measured to the nearest  $\frac{1}{32}$ nd of an inch. The cartons are then drained, shaken out well, and re-weighed to determine the amount of liquid absorbed.

5. (b) *Absorption test at 40° F.*—This test is carried out following the same procedure as described above except for temperature.

In order to secure a wax composition having desirable properties as enumerated above, various processes and compositions have been suggested. For example, it has been suggested that blends of paraffin waxes with micro-crystalline waxes be made which compositions have improved tensile strengths which are desirable. However, it has now been discovered that the impact strength of wax coatings can be greatly increased by blending a narrow cut paraffin wax with a small amount of microcrystalline wax or with polyethylene or both. The microcrystalline wax is added in amounts from about 1% to 10% by weight, preferably from about 2% to 5%, while the polyethylene is added in amounts between 0.1 and 3% by weight.

The polyethylene suitably has a molecular weight between about 4,000 to 22,000. A preferred molecular weight is in the range from about 10,000 to 14,000. With both materials are added, the proportions, based on the narrow cut wax, may be 1-10% of the microwax and 0.1 to 3% of the polyethylene. The paraffin wax to be suitable for this invention must have a boiling point spread not greater than about 50° to 90° F., and preferably not greater than 40° to 60° F., between the 5% to 95% distillation points at 10 mm. pressure. The fact that a narrow cut paraffin wax gives an excellent coating having high impact strength is surprising since the physical inspections lead to the expectation of poor performance. The narrow cut waxes are brittle and have a very low flexibility.

The present invention will be more fully appreciated by reference to the drawing illustrating one embodiment of the same. Referring specifically to the drawing, a waxy crude oil is introduced into distillation zone 1 by means of feed line 2. Temperature and pressure conditions in zone 1 are adapted to remove overhead by means of lines 3 and 4 to low boiling hydrocarbon fractions. A waxy distillate fraction is removed as a side stream by means of line 5, while a residual oil is removed by means of line 6.

The waxy distillate flows through a chilling zone 7 which may comprise a plurality of chilling stages wherein the temperature of the waxy distillate is progressively reduced. A typical operation is to introduce the feed oil into an initial chilling stage at a temperature of about 130° F.; to introduce the feed oil into the second chilling stage at a temperature of about 90° F.; to introduce the feed oil to the third chilling stage at a temperature of about 60° F.; to introduce the feed oil to the fourth chilling stage at a temperature of about 25° F. and to chill the same in the fourth chilling stage to a temperature in the range from about -10 to +10° F. The operation of the respective chilling stages may be varied appreciably and either direct or indirect chilling means utilized. For purposes of illustration, it is assumed that a solvent mixture is used and that the wax-precipitant comprises methyl-ethyl ketone and that the aromatic solvent having a high solubility for oil comprises toluene. It is also assumed that 3 to 4 volumes of total solvent mixture is utilized per volume of waxy oil being dewaxed. The solvent mixture comprises 75% by volume of methyl-ethyl ketone and 25% by volume of toluene.

The entire mixture comprising oily constituents, crystallized wax constituents, toluene and methyl-ethyl ketone, after chilling is held at the filtering temperature and passed to filtering zone 8 wherein the solid wax particles are segregated from the oily constituents by any suitable filtering or separation means. The filtering zone may comprise drum filters, plate and frame presses, centrifuges or suitable equivalent equipment for the separation of the precipitated waxy constituents from the oily constituents.

The oil and a portion of the solvent is removed from zone 8 by means of line 9 and the wax cake washed with a wash solvent introduced into filtering zone 8 by means of line 10. Slack wax and solvent are removed from zone 8 by means of line 11 and passed to a distillation zone 12 wherein a separation is made between the wax and the solvent. It is to be understood that other means of separating the solvent from the wax may be utilized if desirable.

The wax substantially free of solvent is removed from separation zone 12 by means of line 13. The solvent mixture comprising methyl-ethyl ketone and toluene is removed overhead from zone 12 by means of line 14 and preferably recycled to the system. The oil-solvent mixture removed from filtering zone 8 by means of line 9 is introduced into a distillation zone wherein a separation is made between the oily constituents and the solvent mixture.

While the drawing illustrates a solvent dewaxing operation with respect to the production of the slack wax, it is to be understood that the waxy constituents may also be separated in a conventional plate-and-frame pressing operation. The slack wax is further refined to crude scale wax in zone 15, which comprises a conventional sweating operation, or solvent deoiling operation, or the like. The oil removed from zone 15 by means of line 36 may preferably be recycled to zone 7. The scale wax is removed from zone 15 by means of line 35 and may be further refined by treatment with sulfuric acid or fullers earth, bauxite or other absorbent materials, or by hydrogenation under mild treating conditions.

The crude scale wax removed by means of line 35 is either sweated or solvent deoiled to produce a refined wax having an oil content below about .5%, preferably below about .3%. For the purpose of illustration, solvent is introduced by means of line 50. The mixture is introduced into zone 51 wherein the oil content of the wax is reduced so as to produce a refined wax. Solvent is removed by means of line 52 while the refined wax is removed by means of line 53.

This wax is introduced into distillation zone 54 where the same is distilled preferably under pressure of about 10 mm. A discard cut comprising gas oil constituents and contaminants is removed overhead by means of line 55. A low boiling cut is removed by means of line 56, an intermediate or heart cut is removed by means of line 57, while a high boiling cut is removed by means of line 58.

While the distillation range of the refined wax introduced into distillation zone 51 may vary somewhat depending upon the character and the source of the refined wax, a typical paraffin refined wax distillation range at 10 mm. pressure is as follows:

|         | Temperature, ° F. |
|---------|-------------------|
| Initial | 410-435           |
| 5%      | 462               |
| 10%     | 467               |
| 20%     | 475               |
| 30%     | 483               |
| 40%     | 490               |
| 50%     | 499               |
| 60%     | 509               |
| 70%     | 520               |
| 80%     | 532               |
| 90%     | 554               |
| 95%     | 572               |
| Final   | 580-590           |

10 mm. pressure as produced in distillation zone 54 are as follows:

|    |               | Refined Wax Fraction |           |              |
|----|---------------|----------------------|-----------|--------------|
|    |               | Low Boiling          | Heart Cut | High Boiling |
| 10 | Initial, ° F. | 409                  | 449       | 464          |
|    | 5% ° F.       | 434                  | 474       | 496          |
|    | 95% ° F.      | 479                  | 530       | 584          |
|    | Final, ° F.   | 495                  | 539       | 593          |

15 In accordance with the broad concept of the present invention microcrystalline wax or polyethylene is added to these relatively narrow boiling fractions. In accordance with a more specific adaptation of the present invention it is preferred that the microcrystalline wax or polyethylene be added either to the heart cut or the low boiling cut. A particularly desirable wax composition is secured by adding polyethylene or microcrystalline wax to the low boiling fraction, i. e., a fraction having 5% distilled at 10 mm. pressure at a temperature of about 20 430° to 440° F., and having 95% distilled at a temperature from about 475° F. to 485° F.

25 The present invention may be more fully appreciated by the following examples illustrating the same.

30

#### EXAMPLE 1

Two commercial dairy wax compositions characterized by containing 2% of microcrystalline wax were compared with wax compositions of the present invention. The 35 results of the test are as follows:

#### Dairy wax evaluations

| 40 | Wax                                        | Commercial Dairy Wax |        | Narrow Cut #1 |           | Narrow Cut #2 |           |
|----|--------------------------------------------|----------------------|--------|---------------|-----------|---------------|-----------|
|    |                                            | A                    | B      | No additive   | +5% Micro | No additive   | +5% Micro |
| 45 | B. P. Spread -Δ° F. (95-5% Pts. at 10 mm.) | 1129                 | 1112   | 80            | -----     | 65            | -----     |
|    | Wax Consumption lbs./1,000 cartons         | 33.0                 | 33.2   | 35.2          | 35.2      | 34.2          | 34.4      |
|    | Percent Leakers <sup>2</sup>               | 71                   | 69     | 2             | 16        | 5             | 3         |
| 50 | 40° F. Storage <sup>3</sup>                | Satisfactory         | Unsat. | Sat.          | Unsat.    | Sat.          | Unsat.    |
|    | 73° F. Storage <sup>3</sup>                | Satisfactory         | Unsat. | Sat.          | Unsat.    | Sat.          | Sat.      |

<sup>1</sup> Estimated for refined paraffin base.

<sup>2</sup> Cartons are filled with water (colored with methylene blue dye) stored at 40° F. for 16 hours, then dropped, in a standard manner, on one corner. Cartons are then stored for 24 hours and number of leaking cartons counted. Result expressed as number of leakers out of 100 cartons tested.

<sup>3</sup> Cartons are filled with 1% lactic acid in water and stored for 72 hours at both 40° F. and 73° F.

<sup>4</sup> Low boiling fractions. 5% distilled at 420° F. to 440° F.

60 The above data show the surprising fact that the narrow cut paraffin wax itself is highly superior to any commercial wax with regard to the number of leaking cartons obtained after submitting to the test although the storage characteristics are very poor. The data also shows that, while not quite as good as the wax alone as regards percent leakers, the blend of the narrow cut wax #1 (80° F. ΔF. 5-9% pt.) with microcrystalline wax is still much superior to the commercial waxes and is satisfactory in storage. The narrow cut wax #2 (65° F. ΔF. 5-95% pt.) is also far superior to the commercial dairy

65 waxes in leakage resistance although storage is again very poor. However, the addition of microcrystalline wax provides a blend with equally good leakage resistance and fully satisfactory storage characteristics.

70 Other wax blends were prepared in accordance with the present invention and compared to two of the best dairy

Typical inspections of the low boiling fraction, of the intermediate fraction and of the high boiling fraction at

75

wax compositions containing about 2% microcrystalline wax. The results are illustrated in the following table:

composition which comprises blending a refined paraffin wax with about 0.1 to 10% by weight of polyethylene

| Wax                                                           | Commercial<br>Dairy Wax |      | Narrow Cut #1 |              |              | Narrow Cut #2 |              |              |               |                                            |                                        |
|---------------------------------------------------------------|-------------------------|------|---------------|--------------|--------------|---------------|--------------|--------------|---------------|--------------------------------------------|----------------------------------------|
|                                                               | A                       | B    | Alone         | +2%<br>Micro | +5%<br>Micro | Alone         | +2%<br>Micro | +5%<br>Micro | +10%<br>Micro | +3%<br>4,000<br>M. W.<br>Polyeth-<br>ylene | +1%<br>12,000<br>M. W.<br>+9%<br>Micro |
| B. P. Spread —Δ° F. (95-5% pt. at 10 mm.) of<br>base wax..... | 129                     | 112  | 80            | 80           | 80           | 65            | 65           | 65           | 33.0          | 34.3                                       | 34                                     |
| Wax Consumption, lbs./1,000 cartons.....                      | 33.0                    | 33.2 | 33.8          | 33.2         | 33.0         | 35.3          | 34.6         | 34.4         | 3             | 5                                          | 7                                      |
| Percent Leakers.....                                          | 71                      | 69   | 3             | 4            | 16           | 5             | 1            | 3            | 3             | 5                                          | 7                                      |
| 40° F. Storage with 1% Lactic Acid Solution:                  |                         |      |               |              |              |               |              |              |               |                                            |                                        |
| Acid Absorption, lbs./1,000 cartons.....                      | 9                       | 8    | 13            | 15.0         | 10.3         | 15.9          | 8.0          | 6.0          | —             | 7.0                                        | 7                                      |
| Bulge, $\frac{1}{2}$ 2".....                                  | 2                       | 2    | 6             | 8            | 2            | U             | S            | 1            | 2             | 2                                          | 1                                      |
| Overall Storage Rating.....                                   | S                       | S    | U             | U            | S            | U             | S            | S            | S             | S                                          | S                                      |
| 73° F. Storage with 1% Lactic Acid Solution:                  |                         |      |               |              |              |               |              |              |               |                                            |                                        |
| Acid Absorption, lbs./100 cartons.....                        | 16                      | 12   | 18            | 16.8         | 12           | 20.9          | 10.9         | 11           | —             | 11                                         | 8                                      |
| Bulge, $\frac{1}{2}$ 2".....                                  | 7                       | 4    | 10            | 7            | 4            | 13            | 4            | 6            | 4             | 5                                          | 3                                      |
| Overall Storage Rating.....                                   | S                       | S    | U             | U            | S            | U             | S            | S            | S             | S                                          | S                                      |

S—Satisfactory.

U—Unsatisfactory.

What is claimed is:

1. Process for the preparation of an improved wax composition which comprises preparing a refined paraffin wax having an oil content below about 0.5%, segregating from said paraffin wax a narrow boiling fraction having a 5% boiling point at 10 mm. of about 430 to about 440° F. and a boiling point spread of not more than 90° F., between the 5% and 95% points in a 10 mm. distillation, and adding to said narrow boiling fraction about 0.1% to 10% by weight of a material selected from the class of microcrystalline wax, polyethylene having a molecular weight of about 4,000 to 22,000 and mixtures thereof.

2. The process defined by claim 1 in which said added material constitutes polyethylene.

3. The process defined by claim 2 in which said narrow boiling fraction has a boiling point spread of not more than about 50° F. between the 5% and 95% points in a 10 mm. distillation.

4. An improved wax composition consisting essentially of a narrow boiling point refined paraffin wax fraction having a boiling point spread of not more than 90° F. between the 5% and 95% points in a 10 mm. distillation, having a 5% point at about 430 to about 440° F. containing about 0.1% to 10% by weight of a material selected from the class of microcrystalline wax, polyethylene having a molecular weight of about 4,000 to 22,000 and mixtures thereof.

5. The wax composition defined by claim 4 in which the said material contained in the paraffin wax fraction constitutes polyethylene.

6. The composition defined by claim 4 in which the said narrow boiling wax fraction has a boiling point spread of not more than 50° F. between the 5% and 95% points in a 10 mm. distillation.

7. In a process for the preparation of an improved wax

having a molecular weight of about 4,000 to 22,000, the improvement which comprises blending said polyethylene in a narrow boiling refined paraffin wax fraction having a boiling point spread of not more than 90° F. between the 5% and 95% points in a 10 mm. distillation, said fraction having a 5% point of about 430 to about 440° F.

8. In a wax composition comprising a blend of a refined paraffin wax and about 0.1 to 10% of polyethylene having a molecular weight of about 4,000 to 22,000, the improvement which comprises employing for said refined paraffin wax a narrow boiling fraction having a boiling point spread of not more than 90° F. between the 5% and 95% points in a 10 mm. distillation, said fraction having a 5% point of about 430 to about 440° F.

#### References Cited in the file of this patent

#### UNITED STATES PATENTS

|    |           |                        |                |
|----|-----------|------------------------|----------------|
| 40 | 1,937,518 | Henderson et al. ----- | Dec. 5, 1933   |
|    | 2,102,516 | Coster -----           | Dec. 14, 1937  |
|    | 2,348,689 | Abrams et al. -----    | May 9, 1944    |
|    | 2,361,582 | Adams et al. -----     | Oct. 31, 1944  |
| 45 | 2,373,634 | Wagner et al. -----    | Apr. 10, 1945  |
|    | 2,399,521 | Tyler -----            | Apr. 30, 1946  |
|    | 2,443,221 | Bergstein -----        | June 15, 1948  |
|    | 2,467,959 | Bowman et al. -----    | Apr. 19, 1949  |
|    | 2,523,705 | Lovell -----           | Sept. 26, 1950 |
| 50 | 2,559,645 | Larsen -----           | July 10, 1951  |
|    | 2,582,037 | Hyde -----             | Jan. 8, 1952   |
|    | 2,638,459 | Bowman -----           | May 12, 1953   |

#### OTHER REFERENCES

55. "Polythene," E. I. du Pont de Nemours and Co., Inc., Plastic Dept., April 1946, page 22.  
Plastics (Chicago), December 1948, page 12.